

# UNITED STATES PATENT OFFICE.

ROBERT H. AIKEN, OF WINTHROP HARBOR, ILLINOIS.

## PROCESS OF SEPARATING NICKEL FROM MATTES.

No. 800,180.

Specification of Letters Patent.

Patented Sept. 26, 1905.

Application filed March 7, 1903. Serial No. 146,759.

*To all whom it may concern:*

Be it known that I, ROBERT H. AIKEN, a citizen of the United States, residing at Winthrop Harbor, in the county of Lake and State of Illinois, have invented certain new and useful Improvements in Separation of Nickel from Mattes, of which the following is a specification.

My invention relates particularly to the separation of nickel from copper-nickel-sulfid mattes; and its general object is to provide an inexpensive method of obtaining nickel.

More specifically, the object is to combine with the process of my application Serial No. 101,314, "Converting mattes," steps whereby nickel may be separated, as a silicate, from the copper in copper-nickel-sulfid mattes, whether or not the latter contain iron. In the process of that application, which includes certain subprocesses, highly-heated non-molten flux material may be added gradually to molten matte in a converter and the whole subjected to an oxidizing-blast. Where both copper and nickel are present in the matte, the two are not separated from each other by that process. My present process provides for separating the nickel from the copper, as well as eliminating iron and other metals when they are present. In accordance with this latter process a suitable amount of highly-heated flux material, usually silica or silica plus a small amount of lime, (to lower the fusing-point of the silica,) is added to molten matte in a converter, the latter preferably being first highly heated and preferably also provided with a thin non-fluxing lining, the whole being subjected to an oxidizing-blast, when the iron in the matte is oxidized and slagged, and before the nickel and copper are materially acted upon this iron slag is removed from the converter by pouring or otherwise. The completion of this stage is indicated by the change in color of the flame and in the character of the "shots" thrown from the mouth of the furnace, these indications being similar to those observed in the well-understood process of bessemerizing copper-nickel-sulfid mattes. Further blowing, more heated flux material being added, causes the nickel to oxidize and form a nickel-silicate slag, which is also removed from the converter, leaving the copper sulfid. The completion of the second stage is known by indications analo-

gous to those relied upon at the end of the first stage. Still further blowing gives black copper, as in ordinary processes. These three distinct reactions occur in succession through selective chemical action depending upon the various heat tonings in oxidizing the different metals and forming silicates, that action which develops the highest temperature effect being the first to occur. For example, with a matte consisting principally of  $FeS$ ,  $NiS$ , and  $Cu_2S$  we have first the formation of  $FeO$ ,  $SiO_2$ , and gaseous  $SO_2$ . After the completion of this stage, which gives almost perfect elimination of the iron, there is formation of  $NiO$ ,  $SiO_2$ , and  $SO_2$ . After the completion of this second stage and the practically perfect removal of nickel the third and last stage begins, and in this stage the blowing gives  $Cu$  plus  $SO_2$ . It is to be noted that there is a wide difference or decrease in temperature effects in the successive stages. Metallic copper is produced in the last stage, because, as is well known, copper under such conditions will not form a silicate to any appreciable extent so long as sulfur is present. The silica, silica and lime, or other flux material is highly heated and usually added progressively during the process of blowing, but during the first two stages only. The heat produced in blowing the nickel is lower than that produced in blowing on the iron; but the addition of highly-heated flux material not only gives sufficient heat for this stage, but also insures keeping the residue at such a temperature that there is no difficulty in finally finishing the copper.

To determine practically the points at which the iron and the nickel are to be poured off, the operator should be familiar with the different products with which he deals, the color of the flames at the mouth of the converter, and the varying temperature of the bath. The dividing-line between the steps need not be determined with great accuracy, however, for no serious harm results in case either point be passed. In other words, if the iron be not poured off as soon as it is all slagged the nickel that then passes into the slag is recovered in remelting, and similarly when the nickel is all slagged to a silicate no copper silicate will be formed until the copper is blown to a metal, in accordance with the well-known reaction,  $2CuO$  plus  $Cu_2S$  equals  $6Cu$  plus  $SO_2$ . To determine the points in question near enough

for practical purposes, the operator judges by the shots from the mouth of the converter, always indicative of character, by the drop in volume and temperature of the flame, and 5 by changes in the color of the flame. A clearing up of the flame and a clear blue flame, for example, indicate the absence of iron, and a marked drop in the volume of the flame, with a tinge of red, indicate that the nickel is 10 completely slagged. Workmen familiar with the copper-converter processes as carried on in the present state of the art readily understand such indications and find no material difficulty in pouring off at proper times.

15 The nickel silicate or slag produced is comparatively free from other metals owing to the fact that the more freely oxidizable and volatile metals are eliminated during the first stage, while those of greater stability remain 20 with the copper.

The nickel silicate obtained as above set forth is reduced in a suitable furnace by the substitution at high temperature of strong bases, such as CaO and MgO and the reduction 25 of nickel oxid to crude nickel, in this case practically free from metals which would not be readily eliminated by electrolysis.

In the above description the matte has been 30 supposed to contain iron, which was first eliminated. Obviously my invention also includes the separation of nickel from copper-nickel-sulfid mattes originally free from iron or from which the iron may have been removed.

35 The flux used contains not less than seventy per cent. of silica, and hence is hardly fusible at ordinary furnace temperature; but it does not matter whether it fuses or not. The temperature of the added flux need never be 40 above 1,700° centigrade, and it may be far below and even as low as 800° centigrade when the converter and its contents are at a high temperature.

What I claim is—

45 1. The method of separating nickel from copper-nickel-sulfid mattes which consists in adding to molten matte in a converter suitable highly-heated flux material, principally silica, subjecting the whole to an air-blast to oxidize 50 the nickel and removing the nickel-silicate slag thus formed before the blast has materially acted upon the copper.

55 2. The method of separating nickel from copper-nickel-sulfid mattes which consists in adding to the molten matte in a converter highly-heated, non-molten flux material, principally silica, subjecting the whole to an air-blast to oxidize the nickel and removing the nickel-silicate slag thus formed before the 60 blast has materially acted upon the copper.

65 3. The method of separating nickel from copper-nickel-sulfid mattes, which consists in progressively adding to molten matte in a converter highly-heated flux material, prin-

cipally silica, subjecting the whole to an air-blast to oxidize the nickel and removing the nickel-silicate slag thus formed before the blast has materially acted upon the copper. 65

4. The process of separating nickel from copper-nickel-sulfid mattes which consists in adding highly-heated flux material principally silica to molten matte in a converter, subjecting the whole to an oxidizing-blast, removing the iron slag thus formed after approximately all the iron is blown to a silicate, 70 again adding such highly-heated flux material, slagging the nickel, and pouring off the nickel-silicate slag thus formed before the blast has materially acted upon the copper. 75

5. The process of separating nickel from copper-nickel-sulfid mattes which consists in adding highly-heated non-molten flux material principally silica to molten matte in a converter, subjecting the whole to an oxidizing-blast, removing the iron slag thus formed 80 after approximately all the iron is blown to a silicate, again adding such highly-heated non-molten flux material, slagging the nickel, and removing from the converter the nickel-silicate slag thus formed before the blast has 85 materially acted upon the copper.

6. The process of separating nickel from copper-nickel-sulfid mattes which consists in progressively adding highly-heated flux material principally silica to molten matte in a 95 converter, subjecting the whole to an oxidizing-blast, removing from the converter the iron slag thus formed after approximately all the iron is blown to a silicate, again adding 100 progressively such highly-heated flux material, slagging the nickel, and removing from the converter the nickel-silicate slag thus formed before the blast has materially acted upon the copper. 100

7. The method of separating nickel from copper-nickel-sulfid mattes which consists in adding to molten matte in a converter highly-heated flux material containing not less than 105 seventy per cent. of silica, subjecting the whole to an air-blast to oxidize the nickel, and removing the nickel-silicate slag thus formed before the blast has materially acted upon the copper. 110

8. The process of separating nickel from copper-nickel-sulfid mattes which consists in adding highly-heated flux material containing not less than seventy per cent. of silica to molten matte in a converter, subjecting the whole to an oxidizing-blast, removing the iron slag thus formed after approximately all the iron is blown to a silicate, again adding 115 such flux material, slagging the nickel, and pouring off the nickel-silicate slag thus formed before the blast has materially acted upon the copper. 120

9. The method of separating nickel from copper-nickel-sulfid mattes which consists in adding to molten matte in a converter flux

material, containing not less than seventy per cent. of silica, at a temperature between 800° and 1,700° centigrade subjecting the whole to an air-blast to oxidize the nickel and removing from the converter the nickel-silicate slag thus formed before the blast has materially acted upon the copper.

In testimony whereof I have signed my name to this specification in presence of two witnesses.

ROBERT H. AIKEN.

Witnesses:

WALLACE GREENE,  
EDWIN S. CLARKSON.